

## UNITED STATES PATENT OFFICE

2,608,496

COMPOSITION FOR PRODUCING  
PROTECTIVE COATINGSBertha S. Tuttle, Newton, and George E. Jacobs,  
Boston, Mass., assignors to J. N. Tuttle, Inc.,  
Newton, Mass., a corporation of MassachusettsNo Drawing. Application April 1, 1950,  
Serial No. 153,494

4 Claims. (Cl. 148—6.1)

1

This invention relates to protective coatings of the type disclosed in U. S. Patent No. 2,295,063, granted September 8, 1942.

In producing protective coatings of the type disclosed in the above patent it is necessary to observe carefully the various factors which are responsible for imparting a satisfactory coating. So long as the operation is conducted under the supervision of a chemist or one skilled in the art, little if any difficulty is usually encountered, but in many establishments the process is in charge of an unskilled person who does not recognize the development of adverse conditions and unsatisfactory and defective work invariably results.

The principal object of the present invention is to provide a composition which may readily be dissolved in a prescribed amount of water to produce a stable treating solution having the correct pH, solids content, etc., and which does not undergo deterioration or change after a reasonably long period of use, thereby to enable an unskilled operator to practice successfully the above-identified process merely by observing temperature and time of treatment.

Further objects will be apparent from a consideration of the following disclosure which embodies several examples illustrative of our improved composition.

In accordance with the present invention a metallic article having a protective coating consisting essentially of an insoluble porous crystalline surface in the form of an insoluble metal salt of the group consisting of phosphates and oxalates is first subjected to an aqueous solution of sodium aluminate and di-sodium phosphate for a period of from less than five minutes to fifteen minutes or more, depending upon the temperature. The phosphate or oxalate coating may be produced in accordance with the procedures known in the trade as "Parkerizing" and "Bonderizing," which produce phosphate coatings, and the "Loxal" process which produces an oxalate coating.

The preferred composition consists essentially of sodium aluminate and disodium phosphate, although minor amounts of the monosodium salt may be used along with a major portion of the disodium salt as hereinafter illustrated. Sodium borate is also usable as an equivalent of di-sodium phosphate. The ratio of the weight of sodium aluminate to that of the phosphate may vary from about 1:1 to 1:3, but the preferred proportions are of the order of 2:3 of the weight

2

of the sodium aluminate-sodium phosphate mixture. If desired, zinc phosphate



5 may be incorporated in an amount varying from less than 1% to about 10%.

After having subjected the phosphate or oxalate coated article to the treating solution for a period sufficient to cause the composition to react, as described more fully in the above-mentioned patent, the article may then be rinsed in water, dyed in a hot aqueous bath, then rinsed, dried and oiled in conventional manner.

Illustrative compositions are as follows:

15

## Example 1

|                                     | Parts (by weight) |
|-------------------------------------|-------------------|
| Sodium aluminate                    | 5                 |
| Disodium phosphate (anhydrous)      | 6                 |
| 20 Monosodium phosphate (anhydrous) | 1                 |

20

## Example 2

|                                | Parts (by weight) |
|--------------------------------|-------------------|
| Sodium aluminate               | 5                 |
| Disodium phosphate (anhydrous) | 8                 |

25

## Example 3

|                                | Parts (by weight) |
|--------------------------------|-------------------|
| Sodium aluminate               | 5                 |
| Disodium phosphate (anhydrous) | 8                 |
| 30 Zinc phosphate              | 0.24              |

30

The recommended procedure in using any of the above compositions is to dissolve them in about 88 parts of warm water, thereby to provide a treating bath or solution which in use is maintained at a temperature between 120° and 130° F. The phosphate- or oxalate-coated article is dipped in the bath for a period of about five to eight minutes, and then rinsed in water, thereby producing a coating which can be permanently dyed with a wide range of commercially available dyes.

A fast black color is generally difficult to produce, but a chemically coated article treated as above described may readily be colored black by the following treatment:

The article after being rinsed with water is dipped into an aqueous dye bath maintained at or about the boiling point and consisting essentially of 2% Hematin and 1% Fustic. The time of treatment is between five and ten minutes, after which the dyed article is removed, rinsed, dried, and either waxed or oiled. In any case a fast color is not only produced, but also greatly improved rust-resisting properties are imparted.

35

40

45

50

55

The treating composition is quite stable and may be put up in packages or containers which may be kept indefinitely. The composition produces a stable bath having the correct pH when dissolved in the prescribed quantity of water. Hence by merely emptying a packaged amount of the composition in the prescribed amount of water an unskilled operator may make up a reliable treating solution which does not undergo appreciable deterioration for relatively long periods of time. Hence, the usual supervision of a skilled worker may be eliminated.

The present disclosure is for the purpose of illustration and various modifications of the foregoing may be made without departing from the spirit and scope of the invention, as set forth in the appended claims.

We claim:

1. A composition for use in treating chemically coated articles consisting essentially of a mixture of sodium aluminate and disodium phosphate in proportions between 1:3 and 1:1, by weight.

2. A composition for use in treating chemically coated articles, consisting essentially of approximately 5 parts by weight of sodium aluminate, approximately 1 part by weight of monosodium phosphate, and 6 parts by weight of disodium phosphate.

3. A composition for use in treating chem-

ically coated articles consisting essentially of a mixture of sodium aluminate and disodium phosphate in proportions between 1:3 and 1:1, by weight, and up to 10% zinc phosphate, based on the weight of sodium salts.

10 4. A composition for use in treating chemically coated articles consisting essentially of a mixture of about 5 parts by weight of sodium aluminate and about 8 parts by weight of disodium phosphate.

BERTHA S. TUTTLE.  
GEORGE E. JACOBS.

#### REFERENCES CITED

15 The following references are of record in the file of this patent:

#### UNITED STATES PATENTS

| Number    | Name          | Date          |
|-----------|---------------|---------------|
| 1,722,137 | Frischer      | July 23, 1929 |
| 2,102,219 | Raymond       | Dec. 14, 1937 |
| 2,395,126 | King          | Feb. 19, 1946 |
| 2,431,946 | Lurie         | Dec. 2, 1947  |
| 2,478,954 | Tuttle et al. | Aug. 16, 1949 |

#### FOREIGN PATENTS

| Number  | Country       | Date          |
|---------|---------------|---------------|
| 390,249 | Great Britain | Apr. 6, 1933  |
| 390,435 | Great Britain | Apr. 6, 1933  |
| 292,667 | Italy         | Jan. 27, 1932 |